

No. 813,824.

PATENTED FEB. 27, 1906.

E. C. POLLARD.

## SMELTING AND REFINING PROCESS.

APPLICATION FILED MAY 21, 1904.

3 SHEETS—SHEET 1



**WITNESSES:**

*W. B. Fay*  
W. B. Fay.

**INVENTOR**

*Enos C. Pollard*

BY Yannick

ATTORNEYS

No. 813,824.

PATENTED FEB. 27, 1906.

E. C. POLLARD.

SMELTING AND REFINING PROCESS.

APPLICATION FILED MAY 21, 1904.

3 SHEETS—SHEET 2.



WITNESSES:

*John H. Pollard*  
A. E. Tay.

INVENTOR

*Enos C. Pollard*

BY

*Wm. W. Pollard*  
ATTORNEYS

No. 813,824.

PATENTED FEB. 27, 1906.

E. C. POLLARD.

SMELTING AND REFINING PROCESS.

APPLICATION FILED MAY 21, 1904.

3 SHEETS—SHEET 3.

FIG. 5.



FIG. 5.



WITNESSES:

*H. M. Long*  
*A. C. Fay.*

INVENTOR  
E. C. Pollard

BY *M. M. M.*

ATTORNEYS

# UNITED STATES PATENT OFFICE.

ENOS C. POLLARD, OF SEATTLE, WASHINGTON.

## SMELTING AND REFINING PROCESS.

No. 813,824.

Specification of Letters Patent.

Patented Feb. 27, 1906.

Application filed May 21, 1904. Serial No. 209,001.

*To all whom it may concern:*

Be it known that I, ENOS C. POLLARD, a citizen of the United States, and a resident of Seattle, in the county of King and State 5 of Washington, have invented a new and Improved Smelting and Refining Process, of which the following is a full, clear, and exact description.

This invention relates to a novel process 10 for the direct and continuous conversion of ores and matte into a metallic product. It is especially adapted to the sulfid ores of copper, and it may also be employed to special advantage with nickel and copper-nickel 15 ores.

Matte may be treated by the process in the same manner as ores, and hence in the following description and claims the term "ore" 20 may be taken to include matte in such instances as the term "ore" has no special significance.

The prime object of the invention is to bring about not only the smelting of the ores, but the refining or conversion of the matte to 25 produce the finished metallic product by a continuous operation, in which all of the steps are independent and performed in immediate succession, thus making a single concrete process do the work heretofore generally performed by separate processes, and thereby saving in numerous respects, as will be obvious.

In the ordinary process of reducing sulfid ores of copper and other metals—such as 35 those of Butte, Montana, and vicinity, for example—the ore is treated to five separate successive operations before reaching the stage ("blister-copper") that I attain by one. In the first of these operations, that of mechanical concentration to eliminate the large excess of silica occurring in the ore, a great deal of metal is wasted by being carried away in the material thrown out. The most conservative estimates of this waste place it at 40 twenty-five per cent. of the value of metal ultimately recovered. Of course an equal waste of the original gold and silver, which occur in appreciable quantities in these ores, takes place. The copper carried by the tailings is not equally distributed through the mass, but appears in a gradually-increasing percentage, so that were the process of mechanical concentration reduced only the less wasteful part would be performed. If it 45 were reduced one-half, only about one-quar-

ter of the loss would take place. If it were reduced only one-tenth, (or to nine-tenths of its present extent,) the saving would be nineteen per cent. of the total loss or four and three-fourths per cent. of the total amount produced, an amount that would well cover the entire cost of treatment. The amount of silica will be greatly increased also, as well as the amount of iron saved from the pyrites. If we can utilize the fluxing properties of all the iron in smelting and pass a bisilicate slag, (represented, for example, by  $FeOSiO_2$ ), a further saving will be accomplished. The next operation is to roast or calcine the ore, which requires a very extensive plant and 60 some labor and fuel merely to drive off sulfur and oxidize the iron, so as to render it fit to slag off the remaining silica, thereby destroying fuel which in itself would be sufficient to perform the next operation, smelting. Here 65 the iron, which has been oxidized to  $Fe_2O_3$  or  $Fe_3O_4$  is reduced to  $FeO$  at an expense for coke. The matte is allowed to cool and is broken up and remelted in a cupola and is finally taken to the converter. Here the 70 cold air has to be heated to the temperature of the mass, and this entails an additional loss. A large amount of iron which might have served to slag some of the silica must 75 now be slagged by silica taken from the converter-lining. Many experiments have been made to obviate this necessity, the results of which are well known, and the expensive converter-linings are of necessity almost universally used for this purpose. As the process 80 continues the slag accumulates over the matte in the converter until the greater part of the iron is scorified, when it must be removed; otherwise it will foam and fill the entire converter and be expelled from its throat. This 85 foaming is more marked in thin slags and is made use of in an important manner in my new process, as will be seen. When the blast is finished, the total amount of copper found 90 is considerably less than that in the ore 100 at the start. Losses have occurred in the concentration, as was stated above, in the roasting and in the smelting, when the pulverulent nature of the ore permits the blast to carry some of it from the furnace.

It is the main object of my invention to reduce these losses by eliminating the roasting entirely by using more compact material in the furnace and by other steps which will be further pointed out hereinafter. This new 105 110

process will also secure great economy in dispensing with various operations which are expensive and troublesome.

Generally stated, my new process is executed as follows: The ore, with a proper admixture of flux, is fused to produce a matte, and this, with the resultant slag, is drawn off and allowed to settle, the lighter and relatively valueless portions of the slag being run off to the dump, after which the matte and remaining slag is subjected to the action of a blast of air, which bessemerizes the matte, producing a finished metallic product and forcing the metals oxidized by the blast into the slag, and which by its kinetic energy in addition to effervescence produced in a manner to be described is caused to force the slag up into the furnace in which the ore is smelted, the slag there bathing the matte and the silicious component of the ore absorbing a portion thereof and passing off therewith, to be settled as before explained. After once starting the process is kept up continuously, the slag and matte being kept in steady movement so long as operations are to be performed thereon, the ore being continually charged into the melting-furnace, the lighter portions of the slag being steadily drawn off to the dump and the refined or finished metallic product being drawn out of the cycle of operations when the proper degree of refinement is attained.

Reference is to be had to the accompanying drawings, forming a part of this specification, illustrating an apparatus by means of which my invention may be practiced, in which similar characters of reference indicate corresponding parts in all the views.

Figure 1 is a vertical section on the line 1 1 of Fig. 2 of a preferred form of my apparatus. Fig. 2 is a vertical section on the line 2 2 of Fig. 1. Fig. 3 is a sectional plan on the line 3 3 of Fig. 1. Fig. 4 is a vertical section on the line 4 4 of Fig. 3. Fig. 5 is a vertical section on the line 5 5 of Fig. 3.

F indicates the cupola-furnace, C the converter, and B the box or base thereof. S indicates the settler or fore-hearth, and R indicates the receiver for the refined copper or other metal. These parts are supported on a suitable framing which will not be specifically described, since in itself it forms no part of my invention.

F' indicates the boot or bowl at the bottom of the cupola-furnace; and into this the throat of the converter empties.

Reference to Fig. 3 will show that the furnace and converter are transversely elongated, which arrangement I consider best in practice, although it is not essential. From the bottom portion or boot F' of the furnace a passage P extends, (see Figs. 1 and 5,) this passage running downward and discharging into the bottom of the settler at P<sup>3</sup>. A second passage P' passes from the settler at a

point above the discharge or lower end P<sup>3</sup> of the passage P, this passage P' discharging into the lower part of the converter. (See Figs. 1, 2, and 3.) A passage P<sup>2</sup> extends from the bottom of the box or base B into the receiver R. The box or base B is supported on jacks 10 and comprises an outer shell 11, of metal deeply lined with ganister or other non-conducting material 12, supplemented by a thin shell of basic material 13, as magnesite, on the inner surface. 75

14<sup>a</sup> and 14<sup>b</sup> indicate the bostle-pipes for supplying the blast to the twyers 15<sup>a</sup> and 15<sup>b</sup> of the converter. These twyers are arranged just above the box B and in two rows, one at each side of the converter, as best illustrated in Figs. 1 and 3. 80

The converter is divided into two compartments C' and C<sup>2</sup> by two separate dams D and D', the latter and upper one of which is so placed that the two may lap in vertical direction, so as to leave a passage between them for the slag which overflows the dam D. This dam D is composed of a water-jacket covered with non-conducting material supplemented by a basic lining and extends from the highest possible level of the matte, to within a few inches of the bottom, thus allowing the matte which has been blown up to white metal in the compartment C' to settle to the bottom and pass into the compartment C<sup>2</sup>, where it is blown to "blister." The dam D' is composed of a bare water-jacket (as the only molten material to come in contact with it is slag, which will chill and form a non-conducting coating automatically) extending from a point slightly below the top of the dam D to the roof of the converter. The level of the matte in the compartment C' will be several inches lower than that in the compartment C<sup>2</sup> 95 on account of its greater specific gravity. 100

The twyers 15<sup>a</sup> and 15<sup>b</sup> are connected to the separate bostle-pipes 14<sup>a</sup> and 14<sup>b</sup>, which allow of independent regulation of blast-pressure in each set of twyers. 105

The converter is constructed of metallic shells 16, forming a water-jacket completely surrounding the converter and lined with a deep covering 17, of ganister or other non-conducting material, to the upper level of the matte-surface, which lining is supplemented by a thin shell of basic lining. The inner side of the shell 16 has projecting rivets or hooks (indicated at 18) whereby to hold the lining 17 in place. The cupola-furnace is contracted toward its bottom and is formed of inner and outer walls 19, similar to and, if desired, continuations of the walls or shells 16. These walls 19 also form a water-jacket. Above the cupola-furnace is a conduit 20, leading to the stack, and, if desired, rails 21 may be arranged as usual to carry the charging-car, thus permitting the cupola-furnace to be charged from the top in the usual manner. The twyers 23 of the cupola-furnace are lo- 110 115 120 125 130

cated in one row on that side of the furnace opposite the converter and a sufficient distance above the hearth of the furnace to allow of the quiet subsidence of the molten materials.

The settler S is preferably supported on casters 24 and is constructed of a metallic shell 25 at its bottom and inner and outer shells 26 at its sides, forming a water-jacket surrounding the settler. The settler is lined to the level of the bottom of the passage P' with brick 27 or the like and provided with a lid comprising a metallic shell 28 and a brick lining 29.

30 indicates a vertical slot formed in the settler for drawing off the slag, and in this slot is placed a vertically-adjustable dam-plate 31, provided with an orifice 32. By raising and lowering this plate the level at which the slag is allowed to accumulate in the settler may be regulated, it being understood that when the slag reaches the level of the orifice 32 it passes off to the dump.

33 indicates a tap for drawing off the heavier portions of the matte which accumulate in the settler and which lie too low to be passed into the converter through the passage P'. The passages P and P' are formed of inner and outer shells not only constituting the passages, but also forming water-jackets for cooling the same.

34 indicates a removable covering at the top of the passage P, which facilitates introducing an instrument into the passage to clear out clinkers and other obstructions.

The receiver R is formed of a metallic shell 35, lined with non-conducting material 36, such as fire-brick or the like, and this receiver is formed with a vertical slot 37, extending throughout the length of one its walls. This slot is adapted for the passage of the refined product of the apparatus and in operation should be dammed up to the desired height by means of clay or brick. (Indicated at 38 in Fig. 3.) This is protected by a slab of metal 39. The height of this dam in the slot 37 regulates the height of the metal in the receiver R and of the matte and slag in the converter. The blast of course supplied by any suitable blowing-engine, (not shown,) and cold water is caused to circulate throughout the various water-jackets by apparatus which may be of any suitable sort.

The roof of the converter is in sections, which may be easily removed, and consists of a cast-iron shell lined with brick or ganister 40, supported upon hollow cast-iron arches 41, which may be water-cooled. The roof is held in place by keys 42, driven into slots cast in the upper part of the arches 41.

The non-conducting lining of the converter is employed to prevent the low temperature of the water-jacket from chilling the contents of the converter. It is desirable to keep these contents at the highest possible heat,

inasmuch as the molten converter content must furnish the heat to maintain its liquidity and at the same time heat the enormous volume of air passing through it. Further, the reactions take place much more rapidly and effectively at a high temperature. An additional lining of infusible basic material, such as magnesite, which is not attacked by the metallic oxids produced in bessemerizing the matte, is interposed between the silicious lining and the molten contents of the converter in order to protect that silicious lining against the corrosive action of those metallic oxids. The flaring shape of the lower part of the converter operates to preserve the lining against the attack of the metallic oxids by receding from the upward path of the blast, and the oxids therefore ascend to the supernatant layer of slag and are absorbed by that medium, as contradistinguished from being absorbed by the lining of the converter.

I will now explain in specific terms the manner of carrying out the process, using the apparatus above explained. In the following description let it be assumed, for example, that the before-mentioned sulfid ores of copper are being worked. A charge of ore comprising the sulfids of copper, nickel, cobalt, or in some instances lead, together with the sulfid ores of iron and perhaps others, with a silicious slag, is introduced into the furnace F and fused therein. When fuel is mixed with the charge, the fusion is accomplished by the aid of light blasts from the twyars 23. The matte formed by this fusion flows through the passage P into the settler S, filling that portion of the same which lies below the passage P' and overflowing through the same into the converter C. As there is no attempt to eliminate any of the metals in the furnace, this matte will contain all of them, except such as are volatilized. The slag upon fusing follows the course taken by the matte, flowing over the same into the converter. When the level of the matte rises above the twyars 15<sup>a</sup> 15<sup>b</sup>, the blast through these twyars should be turned on. The sulfur in the matte will unite with the oxygen of the blast to form sulfur dioxide, which escapes through the matte and the supernatant layer of slag and passes out through the furnace F. The iron of the matte will unite with the oxygen of the blast to form a base, and this base will unite with the silicious slag to form a basic slag— $FeO + FeOSiO_2 = (FeO)_2SiO_2$ . Such other metals as have greater affinity for oxygen than copper will be eliminated by the bessemerizing blast and pass into the slag as silicates. The material will therefore show a constantly-increasing proportion of copper, (as  $Cu_2S$ ), which will tend to settle toward the bottom. The matte is allowed to rise in the converter to any desired level, provided only that there is sufficient room left below the top of the

passage P' to allow the slag to enter freely. This passage P' may be positioned at any point desired in the converter, and the level of the matte is determined by the height of the dam 38 in the receiver R. The height of the slag in the converter is regulated by the outlet 32. The conversion of the matte is continued in the compartment C' of the converter until white metal (a more or less impure form of cuprous sulfid,  $Cu_2S$ ) settles in the bottom and fills the converter to the level of the bottom of the dam D, thus preventing the passage of lower-grade matte into the compartment C'. There need be no rigid rule as to the exact degree of concentration of this matte, as a small quantity of iron could be oxidized without interfering with the foaming of the slag, for which this separate compartment is especially designed. As a rule, however, it would be better to blow the matte as high as or higher than the white metal in the compartment C'. Subjected to an independently-controlled blast in the compartment C' the remaining sulfur is oxidized and, incidentally, cuprous oxid is formed, which when mixed with cuprous sulfid produces the following reaction:  $2Cu_2O + Cu_2S = 6Cu + SO_2$ . The sulfur dioxide escapes in minute bubbles, causing the slag to foam and occupy greater space, and hence be specifically lighter than the same slag prior to foaming. Experience with converters shows that unless the matte be skimmed of slag when the iron has been entirely oxidized the slag will in a short time occupy from three to four times the space originally occupied. With this device (assuming that there is about eighteen inches of matte above the twyers in the compartment C' and twelve inches of slag above the matte) as soon as the slag occupies more than double its former space it will begin to flow up out of the converter into the furnace F and be poured directly into the melting zone of the furnace, which flow will be accelerated by the kinetic energy or moving force of the upward-flowing blast. In this connection the difference between the kinetic energy and static pressure of the blast should be clearly observed. The static pressure acts equally and tends to raise the level of the slag in the settler above that in the converter and of the matte in the receiver above the matte in the converter. The kinetic energy or moving force of the blast producing an upward current in the converter helps to carry the slag with it in the manner explained. As the slag from the converter enters the cupola it bathes the solid contents of the same, consisting of white-hot silica and such of the sulfids as have escaped fusion. Owing to the low grade of the matte being converted, both slag and gases are at a high heat. The hot basic slag from the converter attacks the hot

silica remaining in the cupola after the fusion of the metallic sulfids and forms a silicious slag  $-(FeO)_2SiO_2 + 2SiO_2 = 2FeOSiO_2 + SiO_2$  or  $(FeO)_2SiO_2 + SiO_2 = 2FeOSiO_2$ . This slag is also acted upon by the molten ferrous sulfid falling through it, cleansing the slag of any copper which may have been scorified in the slag  $-Cu_2OSiO_2 + FeS = Cu_2S + FeOSiO_2$ . The scouring action of this fall of matte also tends to rid the slag of any "shots" or "prills" of matte suspended therein. The matte falling through the slag also causes the bubbles therein to be disrupted, and the slag is thereupon reduced to its original homogeneous or compact state. The hot escaping gases give up their remaining oxygen to the fuel, still further intensifying the heat and fusing the metallic sulfids readily. The slag, together with the matte formed of the molten sulfids, escapes through the passage P into the settler S. I have thus shown that a molecule of  $FeO(SiO_2)$  entering the converter through the passage P' becomes  $(FeO)_2SiO_2$  by the addition of a molecule of  $FeO$ , and then on entering the cupola becomes  $2FeO(SiO_2)$  by the addition of one molecule of  $SiO_2$ , and on entering the settler through the passage P a part of the  $FeO(SiO_2)$  escapes to the dump, while the remainder returns to the converter to be subjected again to the reactions explained. The blister-copper will flow into the receiver R, whence it is drawn off as it accumulates. The lighter portions of the slag run off continually through the outlet 32 to the dump.

After the operation of the process has been started the calculated ore mixture should be regularly charged into the cupola. This mixture should be calculated to produce a silicious slag—that is to say, the silica present in the charge should exceed the amount required to produce a unisilicate when combined with all of the iron and other bases in the charge. In other words, the calculated slag should have the formula  $(RO)_2SiO_2 + SiO_2$ , in which R represents the iron and other metals in the charge other than those to be recovered from the matte produced. The extent of this excess of silica must depend upon local conditions; but there should always be an excess, because the slag passed out to the dump is of the same tenor in silica as that used for fluxing the ferrous oxid in the converter, and good results cannot be obtained by producing a slag in the converter containing a greater proportion of bases than a unisilicate. In order to reduce the reactions to a chemical equation, I have hereinbefore considered the slag discharged to be a bisilicate— $FeO(SiO_2)$ . In fact, this will be a very good slag to adopt in the majority of cases; but I do not confine myself to any specific proportion of silica. The metallic contents of the ore may be any mixture of

the various sulfids of iron and copper often bearing gold and silver in commercially profitable quantities and usually various other metallic sulfids as impurities. In addition to the metallic contents of the ore there may often be cases where lime or other basic flux may be profitably added to the mixture—that is to say, when there is a large excess of silica in the ore. Fuel may be added as the local conditions require. The necessity of a silicious slag presumes a higher temperature than is necessary when a more basic slag is passed. It should be remembered in this connection that an excess of fuel works no evil result beyond a waste of fuel and that according to my process the primary aim is to produce concentration in the converter and use the cupola merely for fusion. Ordinarily in cupola smelting of raw ores a large percentage of the sulfur and iron is oxidized in the furnace, and here an excess of fuel retards the concentration effected. In my process no such condition applies.

It will be noted that the blast-pressure within the converter will cause a homogeneous or compact liquid to rise higher in the receiver R than in the converter; but the metal in the receiver approaches more nearly to metallic copper than that in the converter, and hence it is of greater specific gravity, which will tend to offset the blast-pressure. The blast-pressure will also cause a compact slag to rise a few inches higher in the forehearth than in the converter. This back or static pressure of the blast is due to the obstruction offered by the ore volume in the cupola to the passage of the escaping gases and by no means equals the pressure of the blast as it issues from the tuyers.

The discharge of the slag through the orifice 32 of the settler does not take place immediately upon the entry of the slag into the settler, time being allowed for the slag to settle, and the heavier and richer portions are thus precipitated to the bottom and the lighter and relatively valueless slag passes to the top and escapes to the dump. During the time consumed by this settling operation heat is lost from the slag by radiation and the heating of the water in the jacket; but this loss of heat is divided between the two streams of slag mentioned above, and supposing the two streams of slag to be equal the loss in the escaping stream of slag is only one-half of what it would be were a part of the slag not returned to the converter. This is of great importance in view of the fact that when slag is near its melting-point raising its temperature a few degrees makes a vast difference in its fluidity and the consequent thoroughness with which the matte will separate therefrom. The loss of heat is principally through the walls of the settler, and the slag nearest the walls being cooled below the

temperature of that in the middle of the settler will sink to the bottom and join the stream back to the converter, while the hot central portion rises and escapes, thus further intensifying the heat and consequent liquidity of the escaping stream. In view of the fact that the slags passed in this process are necessarily silicious and that a silicious slag is not only lighter, but separates from the matte more rapidly than a basic slag of the same specific gravity, and, further, that the slag escapes at a higher temperature than is usual, the slags produced by this process are exceptionally clean and free from valuable contents. The heavier portions of the matte with more or less impure lead and lead compounds settle in the bottom of the settler and fill the same to the level of the passage P', whereupon they should be withdrawn by tapping from the hole 33. This forms an independent source of profit.

The contents of the compartment C<sup>2</sup> will be, on the bottom, a layer of metallic copper containing the gold and silver of the ore and some other impurities. This will be distinctly separated from the overlying body of matte, which will be approximately C<sub>2</sub>S, with, perhaps, a small percentage of ferrous sulfid FeS, which percentage will be less near the bottom and away from the dam D. Above this matte there will float a layer of slag, the level of which will be the same as that of the slag in the compartment C', because the two bodies are connected by the passage between the two dams. The level of the matte in this compartment will be lower than that in the compartment C' and will be such that the combined hydrostatic heads of its matte and its slag will balance those in the compartment C'. The receiver R will be filled with metallic copper to a height which will balance the combined pressures of the matte, slag, and blast in compartment C<sup>2</sup>. This pressure and level may be adjusted by raising or lowering the dam-plate 39, while the depth of the layer of slag in the settler S and the compartments C' and C<sup>2</sup> may be adjusted with reference to the level of the matte by raising or lowering the outlet 32. A blast of air is turned on through the tuyers 15<sup>a</sup> and 15<sup>b</sup> of sufficient pressure to penetrate the overlying matte and slag and escape through the body of ore in the furnace F.

While I have illustrated a specific form of apparatus, it is to be understood that I do not limit my invention thereto, but that it may be embodied in many other forms. Although I have described the invention with relation especially to copper ores, it is to be understood that it is not limited thereto, but that others capable of similar action, such as those of the copper group, come within the scope of my invention.

Having thus described my invention, I

claim as new and desire to secure by Letters Patent--

1. A continuous process of bessemerizing mattes, consisting in passing a stream of silicious slag over the bessemerizing regions to absorb the products of bessemerizing blasts, discharging this slag from the bessemerizing region into contact with silicious material to dissolve the silica and incorporate it in the slag, discharging a part of the slag, and returning the remainder of the slag to the bessemerizing regions while still in a molten condition.

2. A process of bessemerizing mattes, consisting in passing a stream of silicious slag over the matte in the bessemerizing regions, discharging the slag from the bessemerizing region into contact with silicious material continuously, discharging a part of the slag, and returning the remainder thereof to the bessemerizing regions.

3. A continuous process of bessemerizing copper mattes, consisting in passing a stream of silicious slag over the bessemerizing regions, discharging this slag into contact with ferrous sulfid to reduce any copper carried by the slag to a subsulfid, discharging a part of the slag, and returning the remainder thereof together with ferrous and cuprous sulfids, to the bessemerizing regions to supply matte to the bessemerizing regions.

4. A continuous cyclical process of reducing ore containing sulfur, consisting in melting it in the presence of a flux to produce matte, separating matte and slag from the ore, passing a stream of slag over the matte, bessemerizing the matte in the presence of the slag, returning a part of the slag to the ore-melting regions to furnish a flux for additional ore, and returning the slag with new matte to the bessemerizing regions.

5. The process of bessemerizing, consisting in passing a stream of silicious slag over the material while being subjected to bessemerizing blasts, causing a mixture of cuprous oxide and cuprous sulfid to react beneath a column of molten slag, thereby causing the formation of sulfur dioxide within the slag and forcing the slag by the dynamic energy due to the effervescence thus produced, together with the kinetic energy of the bessemerizing blasts, into the presence of ore being fused in a higher plane than that from which it was introduced into the converter, and thereafter causing the matte and silicious slag to flow into the bessemerizing region by the force of gravity.

6. A process of bessemerizing consisting in passing a stream of silicious slag over the material while being subjected to bessemerizing blasts, causing a reaction beneath a column of molten slag to produce a gas within the slag and force the latter by the dynamic

energy of effervescence thus produced together with the kinetic energy of the bessemerizing blasts into the presence of ore being fused, and thereafter causing the matte and silicious slag to flow back into the bessemerizing region by the force of gravity.

7. The process of bessemerizing matte, which consists in maintaining over the matte a layer of liquid silicious slag obtained from fusing the ore, passing a blast of air through the matte and through said supernatant layer of slag, and in expelling the slag from the presence of the matte by the combined agency of the kinetic energy of the bessemerizing blast and effervescence due to oxidizing the sulfur in the matte.

8. The process of bessemerizing matte, consisting in passing a stream of silicious slag over the matte in the bessemerizing region, continuously discharging the slag from the bessemerizing region into contact with a silicious material, and returning a part of the slag to the bessemerizing region.

9. A continuous cyclical process of reducing copper ores containing sulfur, consisting in melting them in the presence of a flux to produce matte, separating matte and slag from the ore, passing a stream of slag over the matte, bessemerizing the matte in the presence of slag, drawing off the lighter portion of the slag, returning a part of the slag to the ore-smelting regions in a higher plane than the bessemerizing regions, and returning the slag from the melting regions with new matte to the bessemerizing regions.

10. A process of refining metals, which comprises the fusing of a charge of ore containing sulfur and an excess of silica, retaining all the iron of the ore in the matte, running off and settling the resultant matte and silicious slag, and returning portions of the slag into the presence of the ore.

11. A process of refining metals, which consists in fusing a charge of ore containing copper, iron, sulfur and an excess of silica, without oxidizing the iron and the major portion of the sulfur, running off and settling the resultant matte and slag, and returning portions of the slag into the presence of the ore.

12. A process of refining metals, comprising the fusing of ore containing sulfur; the bessemerizing of the matte produced, and the cyclical circulation of a stream of slag alternately to the fusing and bessemerizing regions.

13. A process of refining sulfid copper ores which comprises fusing the metallic contents of the ore in the presence of a flux and retaining in the matte the iron and the major portion of the sulfur contained in the ore in an unoxidized condition and bessemerizing the resulting material.

14. A process of refining metals which comprises fusing ore containing sulfur, copper and iron, bessemerizing the matte produced, continuously running off the lighter portions of the slag, and cyclically circulating a stream of richer slag alternately to the fusing and bessemerizing regions.

In testimony whereof I have signed my name to this specification in the presence of two subscribing witnesses.

ENOS C. POLLARD.

Witnesses:

RICHARD PENNARD,  
J. L. BELL.